

## UNITED STATES PATENT OFFICE

1,949,801

PROCESS FOR OBTAINING FAST TINTS ON  
WOOLAlbert Landolt, Basel, Switzerland, assignor to the  
firm of Society of Chemical Industry in Basle,  
Basel, SwitzerlandNo Drawing. Application March 7, 1932, Serial  
No. 597,428. In Switzerland March 28, 1931

4 Claims. (Cl. 8—5)

It has been found that valuable, more or less reddish-blue and greenish-blue tints are obtained on wool by first grounding the wool with non-sulfonated arylides of 2:3-hydroxy-naphthoic acid in baths containing free caustic alkali, and under quite definite conditions which will be explained later, and then developing the wool grounded in this manner with such diazo compounds which correspond to the general formula

10



in which the two benzene nuclei bear, besides the  $\text{—N=N—OH}$  group, no other groups occasioning solubility in water or aqueous alkali solutions, such as  $\text{SO}_3\text{H}$ ,  $\text{COOH}$  or  $\text{OH}$  groups. A number of such diazo compounds are disclosed below.

As regards the special grounding conditions, they are dependent on the following circumstances, which partially have been unknown up to now. It is known that caustic alkali affects the wool very easily, especially at raised temperatures and already at moderate concentration. On the other hand it has been found that the arylides of 2:3-hydroxynaphthoic acid, when dissolved in water, with aid of just the sufficient quantity of caustic alkali, have no or only a very slight affinity for wool, but that in the presence of an excess of caustic alkali the affinity for wool increases considerably. This affinity now permits, provided that sufficient alkali is present in the grounding bath, to extensively exhaust the grounding bath, which, on the one hand, has the advantage that no standing baths must be used, and on the other, that by the subsequent coupling on the fiber dyeings are obtained which are fast to rubbing.

It has now been ascertained on the basis of a great number of experiments that the following points have to be considered in order to obtain useful dyeings on the one hand, and to prevent injuring the wool fiber, on the other hand. The proportion of the grounding liquor to the goods ought not to be much smaller than 1:6, and not much greater than 1:50. The grounding bath should not contain more arylide than 5 per cent. calculated on the weight of the wool. Finally, the quantities of sodium hydroxide used should amount to about the 1.5 to 2.5 fold of the weight of the arylide used. Within these extreme combinations the conditions may, of course, vary appropriately according to the existing apparatuses.

The following examples illustrate the invention:—

## Example 1

10 kilos of loose wool are grounded in a liquor containing per 300 litres of water, 0.3 kilo of the para-chloranilide of 2:3-hydroxynaphthoic acid, 1.5 kilo of Turkey red oil, 1.2 litres of caustic soda solution of 36° Bé., 6 litres of sulfite cellulose solution freed from lime of 40 per cent. strength and 6 kilos of sodium chloride. The wool is treated with the circulating liquor for  $\frac{3}{4}$  hour at a temperature of 45° C., then centrifuged and developed in the following developing liquor:—

300 litres of water of 10° C.  
0.3 kilo of the diazo-compound from 4-amino-4'-methoxy-diphenylamine.

0.5 kilo of sodium bicarbonate. The treatment is continued for 20 minutes and the goods are then washed and soured with 0.4 kilo of sulfuric acid in 300 litres of water for 20 minutes at 80° C. In this manner there is obtained a deep, bloomy blue of good fastness to fulling, potting, acid boiling, steaming and light.

When the operation is conducted as prescribed in Example 5 of French specification No. 665,265 there is obtained a feeble, unsightly blue-grey.

## Example 2

For the dyeing of 10 kilos of previously washed loose wool, a dyeing bath is prepared as follows:

0.2 kilo of the  $\alpha$ -naphthylamide of 2:3-hydroxynaphthoic acid made into a paste with sulfuricin or alcohol,

1 litre of caustic soda solution of 36° Bé.  
100 litres of water  
2 kilos of sulfite cellulose waste liquor  
3 kilos of calcined Glauber's salt.

The wool is treated with the circulating liquor for half an hour at ordinary temperature, then removed, centrifuged, and developed in the following bath

0.4 kilo of the diazo-compound from 4'-ethoxy-4-amino-diphenylamine  
0.2 kilo of acetic acid of 40 per cent. strength  
100 litres of water.

The treatment in this bath is to last 20 minutes whereupon the dyeing process is completed as described in Example 1. The wool is dyed a deep blue of good fastness.

## Example 3

20 kilos of wool yarn are moved about for  $\frac{3}{4}$  of an hour, at 45° C., in a dyeing bath consisting of

1000 litres of water

1 kilo of the anilide of 2:3-hydroxynaphthoic acid

5 litres of caustic soda solution of 36° Bé.

20 kilos of sulfite cellulose waste liquor

30 kilos of calcined Glauber's salt.

5 After centrifuging the yarn is developed for half an hour with

4 per cent. of the diazo-compound from 4-amino-4'-methoxy-diphenylamine calculated on 10 the weight of the wool, and

2 per cent. of acetic acid of 40 per cent. strength as described in Example 2. The dyeing process is then completed as described in Example 1. The wool is dyed a deep blue of good fastness.

15 Similar blue tints are obtained with other arylides of 2:3-hydroxynaphthoic acid containing no OH-group in the aryl radicle, such as the anilide, the  $\alpha$ -naphthylamide, the 5- or 4-chloro-2-toluidide, the ortho-, meta- or para-aniside, the ortho- or meta-chloranilide, the meta- or para-toluidide, the 4-chloraniside, the metaxylidide, the ortho- or para-phenetidide, the meta-phenylenediiimide, the toluylenediiimide, the 2:5-dimethoxyanilide or the like.

25 Also more or less greenish or reddish blue tints are obtained with other diazotized 4-aminodiphenylamine derivatives, such as 4-aminodiphenylamine, 4-amino-2'-methoxy-5'-chloro-diphenylamine, 4-amino-2':5'-dimethoxy- or diethoxydiphenylamine or the like.

Particularly advantageous are the substitution products of 4-diazo-diphenylamine whose substituents are alkoxy groups.

What I claim is:-

35 1. A process for obtaining fast tints on wool by means of non-sulfonated arylides of 2:3-hydroxynaphthoic acid containing no OH-group in the aryl radicle and such diazo-compounds which correspond to the general formula



40 in which the two benzene nuclei bear, besides the  $-N=N-OH$  group, no other groups occasioning solubility in water and in aqueous alkali solutions, wherein the wool is grounded in a grounding bath under the following conditions:

(a) proportion of goods to grounding liquor

45 1:5 to 1:50,

(b) the grounding bath does not contain more arylide than 5 per cent. of the weight of the wool to be grounded,

(c) the quantities of sodium hydroxide used correspond to about the 1.5 to 2.5 fold quantity of the arylide used.

45 2. A process for obtaining fast tints on wool by means of non-sulfonated arylides of 2:3-hydroxynaphthoic acid containing no OH-group in

the aryl radicle and such diazo-compounds which correspond to the general formula



80

in which the two benzene nuclei bear, besides the  $-N=N-OH$  group, no other groups occasioning solubility in water and in aqueous alkali solutions, and as substituents at the most two alkoxy groups, wherein the wool is grounded in a grounding bath under the following conditions:

(a) proportion of goods to grounding liquor 1:5 to 1:50,

(b) the grounding bath does not contain more arylide than 5 per cent. of the weight of the wool to be grounded,

(c) the quantities of sodium hydroxide used correspond to about the 1.5 to 2.5 fold quantity of the arylide used.

3. A process for obtaining fast tints on wool by means of non-sulfonated arylides of 2:3-hydroxynaphthoic acid containing no OH-group in the aryl radicle and a diazo-compound corresponding to the formula

85

90

95

100



105

wherein the wool is grounded in a grounding bath under the following conditions:

(a) proportion of goods to grounding liquor 1:5 to 1:50,

(b) the grounding bath does not contain more arylide than 5 per cent. of the weight of the wool to be grounded,

(c) The quantities of sodium hydroxide used correspond to about the 1.5 to 2.5 fold quantity of the arylide used.

4. A process for obtaining fast tints on wool by means of non-sulfonated arylides of 2:3-hydroxynaphthoic acid containing no OH-group in the aryl radicle and a diazo-compound corresponding to the formula

115



120

wherein the wool is grounded in a grounding bath under the following conditions:-

(a) the grounding bath does not contain more arylide than 5 per cent. of the weight of the wool to be grounded,

(b) the quantities of sodium hydroxide used correspond to about the 1.5 to 2.5 fold quantity of the arylide used,

(c) the grounding must be continued until the grounding bath is practically exhausted.

ALBERT LANDOLT.

130

135

80

140

65

145

70

150

75